

# UNITED STATES PATENT OFFICE.

GEORGE D. VAN ARSDALE AND CHARLES G. MAIER, OF NEW YORK, N. Y.

## FLOTATION METHOD.

1,325,817.

Specification of Letters Patent. Patented Dec. 23, 1919.

No Drawing.

Application filed September 25, 1917. Serial No. 193,150.

*To all whom it may concern:*

Be it known that we, GEORGE D. VAN ARSDALE and CHARLES G. MAIER, citizens of the United States, residing at New York, in the county of New York and State of New York, have invented certain new and useful Improvements in Flotation Methods, of which the following is a specification.

This invention is an improvement over present methods of flotation, is applicable to so-called porphyry ores of copper, particularly to those which have heretofore given unsatisfactory recoveries by the ordinary methods of flotation, and has for its chief object the obtainance of greatly increased recoveries.

An example of an ore of this kind is one, which has the following composition.

|                                | Per cent.    |
|--------------------------------|--------------|
| 20 Cu                          | 1.5 to 2     |
| SiO <sub>2</sub>               | 65           |
| Fe                             | 5            |
| Al <sub>2</sub> O <sub>3</sub> | 15           |
| 25 CaO                         | 0.25         |
| MgO                            | 0.75         |
| S                              | 5            |
| Oxid Cu                        | 0.15 to 0.35 |

The large scale operation of flotation has not given satisfactory recovery on this material, the average percentage of copper recovered by flotation based on the total copper in the flotation feed being about 40%. Similar ores from other localities have also yielded low recoveries.

Extensive experiment in variations of the ordinarily recognized variables of the usual flotation practice has not resulted in any very largely improved efficiency, and the same is true for variation in apparatus.

It has been definitely proved that these low recoveries are not due to the character of the copper minerals themselves but to certain constituents of the gangue whose presence in greater or less amounts is responsible for the difficulty.

This is shown by the fact that under strictly parallel conditions of flotation, working by the usual methods, a series of samples, substantially similar as to the characteristics of the copper mineral present, have yielded recoveries varying from 16% to 70%. The average percentage of

copper recovered on this series of samples by ordinary flotation methods was 37%, with 55 average tailings of 1.2%. By operating by our improved method we have obtained an average recovery on the same materials of 79%, with tailings containing 0.4%.

We have also been able to take the tailings 60 from a mill, operating by ordinary flotation methods, carrying 0.73% Cu, and by the application of our improved method reduce the copper therein to 0.36%.

Our invention consists in the discovery 65 that the cause for the low recoveries by flotation on ores of this character is the inherent physical character of a part of the gangue constituents, and in the utilization of this physical character to produce a new and useful effect as a step in a process of flotation, as will be understood from the following description.

The invention has mainly to do with emulsification and the proper control of the same. 75

In the usual descriptions of flotation processes and in many patent specifications, the operation of mixing the oil with the pulp is called emulsification. While it is true that there is no sharp dividing line between emulsions and mere fine subdivision of an oil, it is also true, as can easily be shown, that an oil which is truly emulsified cannot have a selective action for minerals, except when under certain special conditions the mineral 85 itself is the emulsifying agent. Furthermore, the more an oil can be subdivided without becoming emulsified the greater will be its oiling efficiency, and this efficiency will be lessened in proportion to the tendency to 90 true emulsification.

Also it is evident that any condition or reagent producing emulsification will be prejudicial to flotation in proportion to its emulsification efficiency provided this condition of complete emulsification is not removed or destroyed prior to the actual flotation operation. This is the explanation for the injurious action of certain organic materials, such as glue, saponin, tannin, etc. It is also 95 a fact that emulsions of oil can be produced by the action of solid substances known as interfacial substances, which are particles having the property of being wet readily by neither oil nor water.

When an ore contains copper minerals

which under flotation conditions are interfacial, this is not so important, since by sufficient agitation they can be made to emulsify with oil and be subsequently removed, but 5 when the gangue constituent of an ore as distinguished from its mineral constituents which are to be recovered contains any considerable amount of interfacial substances then commercial flotation becomes difficult or 10 impossible; since with ample oil we shall in such a case have a concentrate too low grade to be commercial or else with less oil we shall have a greatly lowered extraction.

Our invention consists in the discovery 15 that the above facts can be utilized to give a greatly improved recovery by first adding oil to a pulp of water and finely ground ore the gangue of which contains inorganic emulsifying constituents, which under ordinary flotation operation are prejudicial to recovery, and then agitating until complete emulsification takes place. In some cases, when working on ores not having enough emulsifying constituents, it may be necessary 20 to add a small amount of an auxiliary emulsifying agent.

Following agitation, which is done solely for the purpose of emulsification and not for mixing in air, we add an agent capable of destroying or removing the condition producing 30 the emulsification and, following this, agitate the pulp until deemulsification takes place and then subject the pulp to the ordinary flotation operation, which may be in any of the apparatus usually employed for 35 the purpose.

By proper choice of the kind and amount of such emulsifying and deemulsifying materials it is possible to attain exactly the 40 conditions needed for successful flotation, and the deemulsification of the oil throughout the pulp insures the completest possible oiling of the mineral particles and consequently the best selectivity.

45 Moreover, the beneficial results of this dual process of deflocculation and subsequent flocculation are not confined only to the oils but also are very important in their relation to the mineral colloids present in 50 the ore. Most ores contain clayey or colloidal portions which adhere strongly to all particles and are a prolific source of low grade concentrates. Now by a process of 55 complete deflocculation of the pulp and subsequent flocculation of the resulting colloidal suspension (which process may be, and is, accomplished by the same reagents and operations used to affect the oils) the clayey portions are first cleaned from the surface of 60 the mineral by being suspended through the pulp, and subsequently re-flocculated, apart from the mineral, leaving the mineral portions of the ore in the cleanest and best possible condition for flotation.

And again, we have discovered that certain ores containing these clayey materials, which have heretofore been so troublesome to the successful flotation of some ores, have the property, in themselves, of stabilizing oil emulsions because the colloidal portions, 65 usually high in alumina, tend to go into the oil-water interfacial surface, (being thereby the cause of the poor recoveries obtained by the usual methods) and that consequently these materials in themselves can constitute 70 the reagents for emulsification necessary for the first step of our process. We may, however, use, in addition, certain other chemical or other emulsifying reagents in order to be better able to control exactly the condition 75 of deflocculation as previously explained.

As an example of our process the following procedure will show the precise steps which must be taken.

A certain ore, containing 2.05% Cu, gives 80 as the best result by the ordinary processes of flotation a recovery of 20.8% and tailings containing 1.87% Cu, due to its extremely clayey character.

We make a pulp containing this ore, finely 85 ground, 1 part to water, 4 parts. To this particular ore we add an amount of sodium hydrate, determined as most suitable by experiment, namely 1 lb. per ton of original ore, and crude petroleum equal to 1% or 90 more of the original ore, and subject this mixture to violent agitation in any suitable or practical type of machine. The object of this agitation is not to produce a froth, and froth cannot be and is not formed thereby, 95 but complete emulsification of the oil and colloidal solids results, without any separation of the metallic mineral constituents. For certain purposes *e. g.* the separation of 100 clay from other materials, a separation of 105 the emulsified portion may be made by adding a frothing agent at this point, and then subjecting to flotation. Ordinarily, however, to further carry out our process this pulp is withdrawn from the emulsifying 110 machine, and there is added thereto a deemulsifying agent, for example an amount of sodium sulfid equivalent to 1.5 lbs. per ton dry ore, this quantity being again determined by careful experiment. The pulp is 115 now agitated until deemulsification of the pulp ensues, and it is then subjected to the ordinary process of flotation in any of the practical types of machines for this purpose. Small amounts of so-called frothing 120 oils may be added during the last stage depending on the type of machine and whether a permanent or evanescent type of froth is desired, but this is not an essential part of the invention as good recoveries may be obtained without any frothing oil whatever.

Under these conditions we have obtained on all copper ores tested a considerably

higher recovery than by the use of the usual flotation methods.

Be it understood, however, that we do not wish to limit our invention to the use of the specific reagents or their relative amounts, as shown above. Any emulsifying agent which may be either originally present in the ore, or added thereto from without at the first stage of the process, may be used in the first step of our method. And, similarly, any deëmulsifying agent is adequate for the second step.

Nor is the sodium sulfid (if this is used) contemplated for the purpose of sulfidizing the oxid copper, as for example in U. S. Patent No. 807,501 granted to Alfred Schwartz, but is used as a deëmulsifying agent. On the contrary this process is intended primarily for the recovery of sulfids from ores carrying considerable clayey gangue, as, for example, the Arizona porphyries. The sodium sulfid and caustic soda are merely cited as specific examples of cheap and convenient reagents which may be used in our process. Furthermore while the example given is applied to copper ore, we do not wish to be limited in the use of the process to such ores, since equally good results may be obtained on other ores, and also as stated the process may be used for removing clay from other minerals for example in an iron ore. Furthermore it should be noted that when caustic is added as an emulsifying agent, the oil used must be a non-saponifiable oil, and there is produced not a soap, but merely a change in the physical distribution of the oil, and also the deëmulsifying agent added does not act chemically but only to again physically change the oil.

In carrying out our process we have found that a suitable oil is fuel oil, say California fuel oil, but other oils may be used, the essential requirement being an oil that can be emulsified under proper conditions and that is not chemically acted on by the emulsifying agent either present in the ore or added to the pulp.

Furthermore we have found that when the amounts of such oils are reduced below the amounts given the recovery percentages are correspondingly reduced. For example, with a quantity of oil equal to 0.5% of the dry ore we obtained a recovery of 32.9% of the total copper, and by increasing the amount of oil to 1.0% we obtained a recovery of 68.5%.

Having thus described the invention, what is claimed as new is:

1. An improved method of ore separation which comprises adding to a pulp of water and ground ore, an emulsifying agent causing true emulsification of the agent so added, in deëmulsifying the agent, and in

then subjecting the treated ore pulp to the 65 operation of flotation to effect separation of the valuable mineral and gangue constituents thereof.

2. An improved method of ore separation which comprises adding to a pulp of water 70 and ground ore containing an emulsifying agent, a substantially insoluble oil capable of forming a true emulsion with the water and the emulsifying constituent of the ore, adding enough of an extraneous emulsifying agent to compensate for any deficiency of such agent contained in the ore, in agitating the pulp thus treated to cause true emulsification, in adding a deëmulsifying agent and re-agitating the pulp until deëmulsification has taken place and the deëmulsified oil has attached itself to the valuable mineral constituents of the ore, and in then subjecting the treated pulp to the operation of flotation to effect separation of the valuable 85 mineral and the gangue constituents.

3. An improved method of ore separation which comprises adding to a pulp of water and finely ground ore, the gangue of which ore contains an inorganic, insoluble emulsifying agent, a substance capable of forming a true emulsion with water and with the emulsifying constituent of the ore, adding enough of an extraneous emulsifying agent to produce true emulsification and to compensate for any deficiency of such agents contained in the ore, and also in a sufficient amount and for the purpose of completely deflocculating any gangue substances mechanically adhering to the minerals, in thoroughly agitating the pulp substantially without introducing air bubbles and without producing a froth until a true emulsification and distribution of the emulsifiable agent and deflocculation of the gangue constituents of the ore is effected, in adding a flocculating or deëmulsifying agent capable of neutralizing or overcoming the deflocculating or emulsifying action of the gangue constituent of the ore and of the deflocculating or emulsifying agent added, in again agitating substantially without the introduction of air bubbles and without producing a froth until flocculation and deëmulsification of the emulsifiable agent and 105 gangue constituents take place and until the deëmulsified agent has attached itself to the valuable mineral constituents of the ore, and in then subjecting the treated pulp to the 110 operation of flotation by any of the usual methods to effect separation of the valuable mineral and the gangue constituents.

4. A step in an improved method of ore separation which comprises adding to a pulp of water and finely ground ore the gangue 115 of which contains an insoluble, inorganic, emulsifying agent, a substantially insoluble substance capable of forming a true emul-

sion with the emulsifying agents of the ore, and incapable of being acted on chemically thereby, and agitating to effect a true emulsification.

5. A step in an improved method of ore separation which comprises adding to a pulp of water and finely ground ore the gangue of which contains an insoluble, inorganic, emulsifying agent, a substantially insoluble 10 substance capable of forming a true emulsion with the emulsifying agent of the ore, and in then adding a sufficient amount of an extraneous emulsifying agent to produce true emulsification and to compensate for 15 any deficiency of such agent in the ore.

6. A step in an improved method of ore separation which comprises thoroughly agitating substantially without introducing air bubbles and without producing a froth, a 20 pulp of water and finely ground ore the gangue of which contains an insoluble, inorganic, emulsifying agent, said pulp also containing a substance capable of forming a true emulsion with water and the emulsifying constituent of the ore, and further containing a sufficient amount of an extraneous emulsifying agent to produce true emulsification and to compensate for any deficiency of such an agent in the ore until 30 true emulsification and distribution of the emulsifiable agent and deflocculation of the gangue constituents of the ore is effected.

7. A step in an improved method of ore separation which comprises thoroughly agitating substantially without introducing air bubbles and without producing a froth, a pulp of water and finely ground ore the gangue of which contains an insoluble, inorganic, emulsifying agent, said pulp also containing a substantially insoluble substance capable of forming a true emulsion with water and the emulsifying constituent of the ore, and further containing a sufficient amount of an extraneous emulsifying agent to produce 40 true emulsification and to compensate for any deficiency of such constituents in the ore until true emulsification and distribution of the emulsifiable agent and deflocculation of the gangue constituent of the ore 45 is effected, in then adding a deemulsifying agent, and in then agitating the pulp until flocculation of the gangue constituents and deemulsification of the emulsifiable agent takes place and until attachment of the emulsifiable agent to the valuable mineral constituents of the ore takes place.

8. An improved method of ore separation which comprises adding to a pulp of water and finely ground ore the gangue of which 50 contains an insoluble, inorganic, emulsifying agent, a substantially insoluble substance capable of forming a true emulsion with water and the emulsifying constituent of the ore, adding a sufficient amount of an extraneous emulsifying agent to produce 55

true emulsification and to compensate for any deficiency of such emulsifying constituent contained in the ore, agitating the mixture to produce true emulsification and deflocculation, adding a deemulsifying agent 70 and again agitating until flocculation of the gangue constituents, and deemulsification of the emulsifiable agent takes place, and until attachment of the emulsifiable agent to the valuable mineral particles has occurred, said mixing being substantially without introduction of air and without the production of a froth, and subjecting the mixture to the operation of flotation by any of the usual methods to effect separation 80 of the valuable mineral and the gangue constituents of the ore.

9. An improved method of ore separation which comprises adding to an ore pulp containing ore constituents capable of truly emulsifying an oil, an oil capable of forming a true emulsion with the water and said ore constituents, in adding sodium hydrate and agitating the pulp to cause true emulsification, in adding sodium sulfid and agitating the pulp to cause complete deemulsification and adhesion of oil to the valuable mineral constituents of the pulp, and in then subjecting the treated pulp to the operation of flotation to effect separation of the valuable mineral and the gangue constituents thereof.

10. An improved method of ore separation which comprises adding to a mixture of water and finely ground ore containing an emulsifying agent, a substantially insoluble oil capable of forming a true emulsion with the water and the emulsifying constituent of the ore, adding enough sodium hydrate to produce true emulsification, in agitating the pulp thus treated to cause true emulsification, in adding sodium sulfid and re-agitating the pulp until deemulsification has taken place and the deemulsified oil has attached itself to the valuable mineral constituents of the ore, and in then subjecting the treated pulp to the operation of flotation to effect separation of the valuable mineral and the gangue constituents.

11. An improved method of ore separation which comprises adding to a pulp of water and finely ground ore, the gangue of which ore contains an inorganic, insoluble emulsifying agent, a substantially insoluble substance capable of forming a true emulsion with water and with the emulsifying constituent of the ore, in adding enough sodium hydrate to produce true emulsification and to compensate for any deficiency 120 of such agent contained in the ore and also in a sufficient amount and for the purpose of completely deflocculating any gangue substance mechanically adhering to the valuable mineral constituent, in thoroughly agitat- 125

ing the pulp substantially without introducing air bubbles or producing a froth until a true emulsification and distribution of the emulsifiable agent and the flocculation of the gangue constituents of the ore is effected, in adding sodium sulfid, in again agitating substantially without the introduction of air bubbles and without producing a froth until deëmulsification and flocculation respectively of the emulsifiable agent and gangue constituents take place and until the deëmulsified agent has attached itself to the valuable mineral constituents of the ore, and in then subjecting the treated pulp to the operation of flotation by any of the usual methods to effect separation of the valuable mineral and the gangue constituents.

12. A step in an improved method of ore separation which comprises adding to a pulp of water and finely ground ore containing an insoluble, inorganic, emulsifying agent, a substantially insoluble substance capable of forming a true emulsion with the emulsifying agent of the ore, and in then adding a sufficient amount of sodium hydrate to produce true emulsification.

13. A step in an improved method of ore separation which comprises thoroughly agitating substantially without introducing air bubbles and without producing a froth, a pulp containing a mixture of water and finely ground ore containing an insoluble, inorganic, emulsifying agent, said pulp also containing a substantially insoluble substance capable of forming a true emulsion with water and the emulsifying constituents of the ore, and further containing a sufficient amount of sodium hydrate to produce true emulsification and to compensate for any deficiency of such emulsifying constituents in the ore, until true emulsification and distribution of the emulsifiable agent and deflocculation of the emulsifying ore constituents is effected.

14. A step in an improved method of ore separation which comprises thoroughly agitating substantially without introducing air bubbles and without producing a froth, a pulp of water and finely ground ore containing an insoluble, inorganic, emulsifying agent and also containing a substantially insoluble substance capable of forming a true emulsion with water and the emulsifying constituent of the ore and further containing a sufficient amount of sodium hydrate to produce true emulsification and to compensate for any deficiency of such emulsifying constituent in the ore, until true emulsification and distribution of the emulsifiable agent and deflocculation of the emulsifying constituent is effected, in then adding sodium sulfid, and in then agitating the pulp until flocculation of the emulsifying constituent and deëmulsification of the emulsi-

fiable agent takes place and until attachment of the emulsifiable agent to the valuable mineral constituents takes place.

15. A step in an improved method of ore separation which comprises adding to a pulp of water and finely ground ore containing an insoluble, inorganic, emulsifying agent, a substantially insoluble substance capable of forming a true emulsion with water and the emulsifying constituent of the ore, a sufficient amount of sodium hydrate to produce true emulsification and to compensate for any deficiency of such emulsifying constituent contained in the ore, agitating the mixture to produce true emulsification and deflocculation, adding sodium sulfid, and again agitating the pulp until flocculation of the emulsifying constituent and deëmulsification of the emulsifiable agent take place and until attachment of the emulsifiable agent to the valuable mineral particles has occurred, said agitating being substantially without introduction of air and without the production of a froth.

16. An improved method of separating emulsifying ore constituents which comprises adding to a pulp of water and finely ground ore, a substantially insoluble substance capable of forming a true emulsion with water and with the emulsifying constituents of the ore, in adding enough of an extraneous emulsifying agent to produce true emulsification of the emulsifiable agent in amount and for the purpose of completely deflocculating the gangue substances mechanically adhering to the valuable mineral content, then thoroughly agitating or mixing the pulp substantially without introducing air bubbles and without producing a froth until true emulsification and distribution of the emulsifiable agent and deflocculation of the gangue and emulsifying ore constituents is effected, effecting deëmulsification, and then separating the valuable mineral and gangue constituents of the ore.

17. An improved method of separating undesirable ore constituents which comprises adding to a pulp of water and finely ground ore, a substantially insoluble substance capable of forming a true emulsion with water and with the undesirable emulsifying constituents of the ore, in adding enough sodium hydrate to produce true emulsification of the emulsifiable agent and to compensate for any deficiency of the emulsifying agent contained in the ore and also in amount and for the purpose of completely deflocculating the gangue substances mechanically adhering to the valuable mineral constituent of the ore, then thoroughly agitating or mixing the pulp substantially without introducing air bubbles and without producing a froth until true emulsification and distribution of the emulsifiable agent.

agent and deflocculation of the gangue and emulsifying ore constituents is effected, effecting demulsification and then separating the valuable mineral and gangue constituents of the ore.

18. An improved method of flotation which comprises adding to a pulp of water and ground ore, a constituent of which latter is an emulsifying agent, an emulsifiable

agent, causing true emulsification of the emulsifiable agent, effecting demulsification and subsequently removing the portion of the pulp comprising the valuable mineral constituent of the ore.

In testimony whereof we affix our signatures.

GEORGE D. VAN ARSDALE. [L. S.]  
CHARLES G. MAIER. [L.S.]